

## UNITED STATES PATENT OFFICE

2,673,387

## ELECTRON EMISSION COATING MIXTURES

Gordon M. Forker, Lyndhurst, Ohio, assignor to  
 General Electric Company, a corporation of  
 New York

No Drawing. Application May 18, 1951,  
 Serial No. 227,115

2 Claims. (Cl. 29—25.14)

**1**  
 My invention relates to electric discharge devices and more particularly to electron emissive cathodes therefor. More particularly my invention relates to compositions of electron emissive coating mixtures useful for activating such cathodes.

My invention is particularly useful in connection with the application of electron emissive coatings to coiled wire cathodes, particularly coiled-coil cathodes as employed in the conventional fluorescent lamps. Such cathodes are composed of a refractory wire, such as tungsten, which is helically wound into a primary coil which is, in turn, helically wound into a secondary coil to constitute the coiled coil. It has been the practice to coat such coils, as by dipping, with an electron emission mixture comprising a suspension of electron emissive material usually comprising alkaline earth carbonates including barium, calcium and strontium carbonates which may be used singly or as double or triple carbonates and which are carried in suspension in a cellulosic ester or ether binder such as a solution of nitro-cellulose in a solvent like amyl acetate. In subsequent manufacturing steps, after the cathode has been sealed in the lamp bulb or envelope, this coating is activated by heating to break down the alkaline earth carbonates to the corresponding oxides, the binder being burned out.

In accordance with the present invention, I have discovered that materially improved results are obtained when the conventional solvent of amyl acetate is replaced by "Cellosolve" acetate (ethylene glycol monoethyl ether acetate).

One of the advantages of employing "Cellosolve" acetate as the solvent in place of amyl acetate is that it makes a more stable mixture because of its slower evaporation rate (21 compared to 62 on an arbitrary scale where butyl acetate is set at 100). The amyl acetate mixtures require frequent dilution as the solvent evaporates. The necessity of dilution is evidenced by a bridging of the emission mixture across the secondary coils of the coiled-coiled cathodes. However, each dilution is likely to go too far, with the result that the coil then is not filled with a proper weight of the emission mixture. Another disadvantage of mixtures employing amyl acetate is that they tend to form crusts on the coating equipment, such as that disclosed in Patent 2,545,909 to W. P. Zabel, which is assigned to the assignee of the present invention.

Even more important, and wholly unexpected,

**2**  
 advantages of employing "Cellosolve" acetate as the solvent are found in the improved character, as well as the heavier weight of the filling of the electron emissive mixture in the cathode coil. 5 In a given size coil, the weight of the emissive material is increased from an average of about 4.5 mg. to about 5 mg. for "Cellosolve" acetate mixes as compared with amyl acetate mixes. However, even aside from the increased weight, 10 it is noticeable that the "Cellosolve" acetate mix penetrates into, and more completely fills, the primary coil of the cathode. The material within the primary coil is fully effective and is retained for a long useful life, whereas any material left 15 hanging on the outside of the coil becomes dislodged and falls off during operation of the lamp containing the cathode. The improved character of the fill or "coating" is evidenced by the fact that the primary coil contains a higher proportion of solid slugs of the emission material and a lower proportion of annular segments. 20 These results may be due, in part, to the fact that since the "Cellosolve" acetate requires more time to evaporate, it gives the mixture time to sink deeper into the primary coil before it freezes 25 or sets. However, it is also fact that other solvents, even some having slower evaporation rates than "Cellosolve" acetate, such as diacetone alcohol and acetonyl acetone, are not satisfactory. 30 I have obtained good results by employing mixtures comprising a suspension of about 130-260 grams of alkaline earth carbonates in about 115 to 145 ml. of a binder of nitrocellulose dissolved in "Cellosolve" acetate and having a 35 viscosity of about 30-100 centipoises. I prefer to employ triple carbonates of barium, strontium and calcium. The composition of the triple carbonate may be varied widely but good results have been obtained with proportions of 40 approximately 38.6 mole per cent barium, 31 mole per cent strontium and 30.4 mole per cent calcium.

A specific example, by way of illustration, of a mixture with which good results have been obtained is the following:

The binder is prepared by mixing 2.1 kg. of nitrocellulose with 147 kg. of "Cellosolve" acetate and rolling the mixture until the solution is complete. The solution is then filtered, checked for a solid content of 0.5-1.5 per cent and a viscosity of 30-33 seconds at 25° C. in a #7 duPont cup, and adjusted if necessary. A mixture is then made of 17.04 liters of the aforesaid binder with 30 kg. of triple carbonates of the alkaline earth metals. This mixture may be ball-milled

for approximately 20 hours. The mixture is then stored until ready for application to cathodes in any suitable manner such as that disclosed in the aforesaid Patent 2,545,909.

What I claim as new and desire to secure by Letters Patent of the United States is:

1. A coating composition for coiled-coil cathodes and consisting essentially of a suspension, in proportions corresponding to the stated amounts, of about 130 to 260 grams of finely 10 divided alkaline earth carbonates in about 115 to 145 ml. of a binder of nitrocellulose dissolved in ethylene glycol monoethyl ether acetate and having a viscosity in the range of about 30 to 100 centipoises.

2. The method of introducing activating alkaline earth materials on cathodes in electric discharge devices which comprises suspending powdered alkaline earth metal carbonate in a binder of nitrocellulose dissolved in ethylene 20 glycol monoethyl ether acetate in proportions corresponding to about 130-260 grams of carbonate in about 115-145 ml. of a binder of nitro-

cellulose dissolved in ethylene glycol monoethyl ether acetate and having a viscosity in the range of about 30-100 centipoises, coating a coiled-coil cathode with said suspension, sealing the cathode in said device, and activating the cathode by heating to break down the alkaline earth carbonate to the corresponding oxide and to burn out the binder.

GORDON M. FORKER.

References Cited in the file of this patent

UNITED STATES PATENTS

| Number    | Name        | Date          |
|-----------|-------------|---------------|
| 1,791,301 | Davidson    | Feb. 3, 1931  |
| 1,842,161 | Frederbaugh | Jan. 19, 1932 |
| 2,083,372 | Guthmann    | June 8, 1937  |
| 2,223,977 | Wamsley     | Dec. 3, 1940  |

OTHER REFERENCES

"Handbook of Material Trade Names," Zimmerman and Lavine 1946 pg. 95, Industrial Research Service, Dover, N. H.